

## UNITED STATES PATENT OFFICE.

WILLIAM G. CALKINS, OF DETROIT, MICHIGAN, ASSIGNOR TO CHRYSLER CORPORATION, OF HIGHLAND PARK, MICHIGAN, A CORPORATION OF DELAWARE.

## HYDRAULIC-BRAKE SOLUTION.

No Drawing.

Application filed October 9, 1928. Serial No. 140,686.

This invention relates to a low vapor pressure, high boiling point solution and more particularly to a solution adapted for use in a closed hydraulic system such as is commonly used in a closed hydraulic brake system.

In closed hydraulic brake systems of the type which operate on automobile vehicles, it is difficult to maintain a constant pressure within the system at all temperatures, due to vaporization and condensation of the solution used. Certain portions of the system may be exposed to heated parts of the vehicle, so as to absorb heat therefrom, as for example, one of the lines leading to the brake operating mechanism may be adjacent the muffler or motor. This and other heat, used on frictional heat from the brake drum, causes vaporization of the ordinary solution, creating a pressure in the entire system which locks the brakes. Changes in atmospheric pressure cause changes in the pressure when a low boiling point solution is used.

It is therefore an important object of this invention to provide a solution having a high boiling point.

Certain hydraulic brake systems have their operating parts made of steel, their connecting lines usually are made of copper tubing, and where flexibility is required, rubber hose is commonly used. The operating parts require lubrication and to lubricate these parts by the solution used in the system, it is necessary to provide a solution which has no corrosive effect on other parts of the system such as rubber and copper. Light mineral oils are objectionable in that they attack the rubber and cause deterioration thereof.

Another object of this invention is to provide a solution having lubricating qualities which will have no corrosive effect on the parts of the system.

A vegetable oil such as castor oil has been found to be most satisfactory, but due to its viscosity when used without dilution, it is not desirable for exceedingly low temperatures. It therefore becomes necessary to dilute the castor oil with a liquid of less viscosity and as before mentioned one hav-

ing a high boiling point and no effect on the parts of the system.

Any of the higher alcohols or their derivatives, such as butyl, iso butyl, amyl, iso amyl, prophyl, iso prophyl, et cetera, have a boiling point at atmospheric pressure higher than 80° centigrade. The boiling points of these alcohols range from 82° centigrade, iso propyl, to 137.8° centigrade, normal amyl. Normal butyl alcohol,  $\text{CH}_3(\text{CH}_2)_2\text{CH}_2\text{OH}$ , has a boiling point of 117° centigrade and when used to dilute the castor oil a non-corrosive solution is produced which has lubricating qualities and vaporizes only at a temperature above unusual conditions.

While amyl alcohol,  $\text{CH}_3(\text{CH}_2)_3\text{CH}_2\text{OH}$ , has a boiling point of 137.8° centigrade it causes the sulphur in the rubber connections of the system to attack the copper tubing forming a black copper sulphide corrosion within the system. Through a series of tests butyl alcohol has been found most desirable as it has less action on the parts of the system, its boiling point is sufficiently high to prevent vaporization under extraordinary condition, and it is a more commercial product.

It has been found that a solution consisting approximately of 50% castor oil and 50% of one of these higher alcohols, particularly butyl alcohol, makes a desirable solution. Where butyl alcohol is used, the solution has a boiling point of 117° centigrade or 242° Fahrenheit as compared to 76° centigrade, 170° Fahrenheit, when ordinary denatured alcohol is used; the latter being undesirable.

It is to be understood that while butyl alcohol has been found to be the most satisfactory to meet the requirements for a solution used in a system of the class described, other derivatives of the higher alcohols may be used when the parts of the system are not subject to corrosion and exceedingly high temperatures are present and it is not my intention to limit the scope of this invention other than by the terms of the appended claims.

What I claim is:

1. A hydraulic solution composed of castor oil and butyl alcohol.

100

2. A hydraulic solution composed of approximately fifty percent castor oil and approximately fifty percent butyl alcohol.
3. A hydraulic solution composed of castor oil and a monohydric alcohol having a boiling point above 80° C. at atmospheric pressure.
4. A hydraulic solution composed of approximately fifty percent castor oil and approximately fifty percent of a monohydric alcohol having a boiling point above 80° C. at atmospheric pressure.
5. A hydraulic solution composed of castor oil and an alcohol of the monohydric series having a boiling point not less than 117° C. at atmospheric pressure.

WILLIAM G. CALKINS.